

# UNITED STATES PATENT OFFICE.

ROBERT ABBOTT HADFIELD, OF SHEFFIELD, ENGLAND.

## PROCESS FOR IMPROVING THE MAGNETIC QUALITIES OF IRON-SILICON-MANGANESE-ALUMINIUM ALLOYS.

1,086,766.

Specification of Letters Patent.

Patented Feb. 10, 1914.

No Drawing. Application filed March 21, 1907, Serial No. 363,664. Renewed June 27, 1913. Serial No. 776,172.

*To all whom it may concern:*

Be it known that I, ROBERT A. HADFIELD, a subject of the King of Great Britain and Ireland, residing at Parkhead, Sheffield, England, have invented a certain new and useful Improvement in Processes for Improving the Magnetic Qualities of Iron-Silicon-Manganese-Aluminium Alloys, of which the following is a specification.

10 In U. S. Letters Patent No. 745,829, granted to me December 1, 1903, I have described and claimed a process of producing a magnetic material of high permeability and low hysteresis action which consists in alloying a magnetic body with silicon, heating the alloy to a relatively high temperature below its melting point, allowing the alloy to cool, reheating it to a temperature below that first employed and allowing to cool slowly.

In U. S. Letters Patent No. 842,403, dated January 29, 1907, I have described an alloy containing iron, silicon, manganese and aluminium in the following proportions, to wit: silicon from 2 to 4.5%, manganese not exceeding .7% and aluminium not exceeding 1.3%.

My present invention is a process of increasing the permeability and electric resistance, and decreasing the hysteresis action of the said iron-silicon-manganese-aluminium alloy. I carry my said process into effect by melting together the ingredients in a suitable vessel, casting into ingots, rolling or working and treating the same by first heating the alloy to between 900° and 1100° centigrade, then allowing it to cool, then reheating to between 700° and 850° centigrade, that is, to a temperature lower than the one attained during the first heating and finally allowing the alloy to cool slowly.

I claim:

1. The herein described process of obtaining an iron silicon manganese aluminium alloy of high magnetic permeability and electric resistance and low hysteresis action which consists in heating said alloy to a high temperature above 900° C. but below its melting point, allowing the alloy to cool slowly, reheating the alloy to a second high temperature but below about 850° C. and then allowing it to cool slowly.

2. The process of producing a magnetic alloy of high permeability and electric resistance and low hysteresis action which consists in alloying iron with silicon from about 2 to about 4.5%, manganese not exceeding about .7% and aluminium not exceeding about 1.3% then heating said alloy to a temperature ranging from about 900° C. to below 1100° C. then allowing the alloy to cool, then reheating the alloy from a temperature ranging from about 700° C. to not over 800° C. and then finally cooling.

3. The herein described process of producing a magnetic alloy of high permeability and low hysteresis action which consists in alloying iron with silicon from about 2 to about 4.5%, manganese not exceeding about .7% and aluminium not exceeding about 1.3%, then heating said alloy to a high temperature above about 900° C. but below its melting point, then allowing the alloy to cool slowly, then reheating the alloy to a high temperature not substantially above 850° C. and finally allowing it to cool slowly.

4. The herein described process of producing a magnetic alloy of high permeability and low hysteresis action which consists in alloying iron with silicon above about 2%, manganese not above about .7% and aluminium not above about 1.3%, then heating the alloy to above about 900° C., then cooling, then reheating the alloy to below about 850° C. and finally cooling.

5. The herein described process of producing a magnetic alloy of high permeability and low hysteresis action which consists in alloying iron with silicon above about 2%, manganese not above about .7% and aluminium not above about 1.3%, then heating the alloy to above about 900° C., then cooling slowly, then reheating the alloy to below about 850° C. and finally cooling.

In testimony whereof I have affixed my signature in presence of two witnesses.

ROBERT ABBOTT HADFIELD.

Witnesses:

HUGH HUGHES,  
Wm. O. BROWN.